

# United States Patent [19]

Inoue

[11] Patent Number: 4,626,488

[45] Date of Patent: Dec. 2, 1986

[54] **POLYMERIC BINDER FOR TONER HAVING SPECIFIC WEIGHT DISTRIBUTION**

[75] Inventor: Sukejiro Inoue, Yokohama, Japan

[73] Assignee: Canon Kabushiki Kaisha, Tokyo, Japan

[21] Appl. No.: 714,520

[22] Filed: Mar. 21, 1985

[30] **Foreign Application Priority Data**

Apr. 28, 1984 [JP] Japan ..... 59-86767

[51] Int. Cl.<sup>4</sup> ..... G03G 9/08

[52] U.S. Cl. ..... 430/109; 430/126;  
430/904

[58] **Field of Search** ..... 430/109, 99, 126, 904

[56] **References Cited**

**U.S. PATENT DOCUMENTS**

4,486,524 12/1984 Fujisaki ..... 430/109

*Primary Examiner*—John L. Goodrow  
*Attorney, Agent, or Firm*—Fitzpatrick, Cella, Harper & Scinto

[57] **ABSTRACT**

A toner for developing electrostatic image excellent in harmonization of hot roller fixability, anti-offset characteristic and durability is provided by melt-kneading a binder resin and a colorant and pulverizing the kneaded product. The binder resin comprises a polymer having at least three peaks or shoulders in its chromatogram obtained by gel permeation chromatography, wherein the at least three peaks or shoulders include a peak or shoulder A having the largest molecular weight Ma of 2,000 to 80,000, a peak or shoulder C having the smallest molecular weight Mc satisfying, the relationship of  $Mc/Ma \geq 150$ , and a peak or shoulder B having an intermediate molecular weight between the Ma and Mc.

**34 Claims, 1 Drawing Figure**



**POLYMERIC BINDER FOR TONER HAVING  
SPECIFIC WEIGHT DISTRIBUTION**

**BACKGROUND OF THE INVENTION**

The present invention relates to a toner binder resin for a dry-system developer for use in electrophotography, electrostatic printing, magnetic recording, etc., a toner containing the binder resin and processes for producing the binder resin and the toner.

Heretofore, as electrophotographic processes, a large number of processes have been known, including those disclosed in U.S. Pat. No. 2,297,691; and Japanese Patent Publication Nos. 23910/1967 and 24748/1968. These processes comprise the steps of forming an electrical latent image on a photosensitive member generally comprising a photoconductive material, subsequently developing the latent image with a toner, and optionally transferring the resultant toner image onto a transfer material such as paper and fixing the toner image by means of heat, pressure, solvent vapor, etc., thereby to obtain a copy. Where the step for transferring the toner image is included, there is also provided a step for removing residual toner.

Further, several developing methods have been known for visualizing electrical latent images, such as the magnetic brush method as disclosed in U.S. Pat. No. 2,874,063, the cascade developing method as disclosed in U.S. Pat. No. 2,618,552, the powder cloud method as disclosed in U.S. Pat. No. 2,221,776, and a method using an electroconductive magnetic toner as disclosed in U.S. Pat. No. 3,909,258.

The toner used in these developing methods conventionally comprises fine particles of a natural or synthetic resin and a dye or pigment dispersed therein. For example, fine particles with a size of the order of 1 to 30 $\mu$  obtained by micropulverizing an intimate mixture of a binder resin such as polystyrene and a colorant dispersed therein, have been used as a toner. A magnetic toner is one containing particles of a magnetic material such as magnetite. In a system using a so-called two-component developer, a mixture of such a toner with carrier particles such as glass beads or iron powder is ordinarily used.

For the toner, although various physical and chemical properties are required, most known toners have a number of defects as explained hereinbelow. Thus, many of the toners readily fusible upon heating are liable to solidify or agglomerate during storage or in a copying machine. Many toners have poor triboelectric characteristics and poor free-flowability due to temperature change in the environment. Further, in the continuous use of many toners involving repetitive development, the density of the image is changed or the background density increases due to mutual deterioration of the toner, carrier particles and photosensitive member through collision between the toner particles and carrier particles, and contact between these particles and the photosensitive member. Further, many toners ordinarily cause background density to increase, resulting in so-called fogging, when it is actually intended to increase the density of copied images by increasing the amount of toner attached to the photosensitive member having a latent image.

One of these undesirable phenomena is caused by the fragility of a toner. That a toner is fragile means that the toner is readily pulverized by a mechanical power and is a desirable feature from the viewpoint of the productiv-

ity of a toner. However, a fragile toner is readily pulverized into fine powder even under a normal load applied thereto in a developing apparatus, thereby to cause undesirable phenomena such as fogging through contamination of carrier particles, soiling of a developer sleeve, and imperfect charge controlling characteristic of the toner particles per se. Thus, the fragility of a toner significantly affects the life of the developer. In order to obviate such deterioration, it is conceivable to use a polymer of a high molecular weight as a binder resin for the toner. However, use of such a high-molecular weight polymer is not desirable from the viewpoint of economization of energy consumption, because it requires a larger amount of heat due to elevation of a fixation temperature when the ordinary heat-fixation of images is carried out in the final step of the copying process. Further, in order to remove this drawback, it has been proposed to add a small amount of plasticizer into a toner, but such a proposal has not been necessarily successful because it is accompanied with problems such as decrease in free-flowability of the toner and contamination of the carrier particles. On the other hand, if a toner is too hard, practical production thereof becomes difficult because mechanical pulverization becomes nearly impossible.

For the above reasons, polystyrene, a styrenebutyl methacrylate copolymer or the like of a relatively low molecular weight of the order of several thousands having an appropriate hardness or rigidity has heretofore been used as a binder resin for toner. On the other hand, manufacturers are trying to produce copying machines and toners having decreased, or maintenance free, operation. It has been determined that, under these conditions, a relatively low molecular-weight polystyrene or styrene-butyl methacrylate copolymer is not sufficient in hardness, and a material with a higher hardness is required. Further, this class of ordinary binder resin is not especially suited for heat fixation by means of hot rollers which are the most widely adopted fixing means. More specifically, the binder resin is best adapted for giving a toner with good fixation characteristic, i.e., good adhesion thereof to a transfer medium such as paper through fusion of the binder on heating and pressure-application. However it is difficult to obviate the soiling of the heat rollers due to sticking of the toner onto the rollers, i.e., so-called offsetting. For this reason, silicone oil has been applied by adding a complicated mechanism, although such a measure is not completely satisfactory for removing offsetting and is disadvantageous from the points of cost as well as maintenance. Thus, development of a toner binder free of such a problem is desired. Several measures have been previously proposed, including changing binder components in various manners, various means such as crosslinking and others for adjusting the molecular weight of binder. There has also been adopted a measure of incorporating an additive such as a low-molecular weight polyolefin or another plasticizer into a toner. The incorporation of such an additive is, however, accompanied with various problems such as poor dispersibility with the binder, impairment of free flowability of the toner powder and the promotion of toner agglomeration, and a satisfactory additive has not been found so far.

As explained hereinabove, improvement of toner performances by the use of additives is limited, and improvement of the resin component which is a principal binder component is believed to be the most impor-

tant. There have been some proposals of adjusting the molecular weight of a binder resin. These proposals are not more than saying that it is desired to broaden the molecular weight distribution by applying crosslinking and do not clarify what range of molecular weight distribution is desirable. The proposals made heretofore refer to a binder resin having a single peak in the molecular weight distribution and having an average molecular weight in a certain range, or to a binder resin further defined by a broadness of the molecular weight distribution in terms of a dispersion (more specifically, a ratio  $(M_w/M_n)$  of weight-average molecular weight ( $M_w$ )/number-average molecular weight ( $M_n$ ) obtained by gel permeation chromatography (hereinafter, sometimes abbreviated as "GPC"). However, none of this category of binder polymers satisfies the overall requirements, particularly the overall fixation performances, including various characteristics as described hereinabove required for heat-fixable dry-system developers.

Further, binder resins having a molecular weight distribution satisfying certain relationships have been proposed. For example, Japanese Patent Laid-Open Applications Nos. 16144/1981 and 82258/1983 propose methods for improving the fixing characteristics of a toner by mixing a plurality of binder resins having different molecular weight ranges. Especially, Japanese Patent Laid-Open Application No. 82258/1983 discloses a binder having three peaks in the molecular weight distribution, which gives an improvement in the fixing characteristics. However, a binder resin only comprising three components of different molecular weights does not provide a satisfactory combination of fixability and anti-offset property on heat-fixation by means of heat rollers but still involves some problem in durability.

#### SUMMARY OF THE INVENTION

An object of the present invention is to provide a binder resin for toner free of the above-mentioned defects of the conventional toners and giving a toner with excellent physical and chemical properties, a toner containing the binder resin and processes for producing the same.

Another object of the present invention is to provide a binder resin for toner suitable for fixation by hot rollers, a toner for hot roller fixation containing the binder resin, and processes for producing the same.

A still further object of the present invention is to provide a toner binder resin for giving a toner excellent in overall characteristics on hot roller fixation, i.e., combination of characteristics such as capability of being fixed at a relatively small amount of heat, substantial freeness from offsetting to hot rollers, and capability of realizing smooth discharge of paper, a toner containing the binder resin, and processes for producing the same.

A still another object of the present invention is to provide a binder resin capable of giving a toner excellent in impact resistance, free-flowability without causing agglomeration and excellent in durability, a toner containing the binder resin, and processes for producing the same.

A further object of the present invention is to provide a binder resin for giving a toner less-sticky to related members such as a carrier, a toner holding member, a photosensitive member and a cleaning blade and giving

less damage to the related members, a toner containing the binder resin, and processes for producing the same.

A still further object of the present invention is to provide a binder resin for giving a toner capable of producing constantly stable clear images free of fogging, a toner containing the binder resin and processes for producing the same.

As a result of my further study, it has been found that a binder resin having a molecular weight as well as a molecular weight distribution which are more specific than those of the known binder resins is effective for accomplishing the above objects. Particularly, I have found that it is not necessarily sufficient for a binder resin to have at least three peaks or shoulders in its molecular weight distribution curve as exemplified in the above-mentioned Japanese Patent Laid-Open Application No. 82258/1983, and that it is critical that the binder resin has a sufficient molecular weight distance between the peaks corresponding to the largest and smallest molecular weights among the at least three peaks or shoulders.

Thus, according to one aspect of the present invention there is provided a binder resin for a toner comprising a polymer having at least three peaks or shoulders in its chromatogram obtained by gel permeation chromatography, wherein the at least three peaks or shoulders include a peak or shoulder A having the smallest molecular weight  $M_a$  of 2,000 to 80,000, a peak or shoulder C having the largest molecular weight  $M_c$  satisfying, the relationship of  $M_c/M_a \geq 150$ , and a peak or shoulder B having an intermediate molecular weight between the  $M_a$  and  $M_c$ .

The present invention further provides a toner comprising a colorant and a binder resin, the binder resin comprising a polymer having at least three peaks or shoulders in its chromatogram obtained by gel permeation chromatography, wherein the at least three peaks or shoulders include a peak or shoulder A having the smallest molecular weight  $M_a$  of 2,000 to 80,000, a peak or shoulder C having the largest molecular weight  $M_c$  satisfying, the relationship of  $M_c/M_a \geq 150$ , and a peak or shoulder B having an intermediate molecular weight between the  $M_a$  and  $M_c$ .

The present invention according to another aspect thereof, provides a process for producing the binder resin for a toner as mentioned above, comprising; subjecting a mixture of a vinyl monomer and a crosslinking monomer to solution polymerization in an organic solvent capable of dissolving the polymerization product of the mixture in the presence of a polymerization initiator having a 10 hour - half life temperature of 100° C. or higher.

The present invention further provides a process for producing the binder resin for a toner as mentioned above, comprising: uniformly mixing a polymer having a weight-average molecular weight of  $1 \times 10^3$  to  $8 \times 10^4$ , a polymer having a weight-average molecular weight of  $3 \times 10^5$  to  $10^6$  and a polymer having a weight-average molecular weight of  $3 \times 10^6$  or larger.

The present invention, according to still another aspect thereof, provides a process for producing a toner, which comprises: melt-kneading a colorant and the above-mentioned binder resin, cooling the resultant mixture, and pulverizing and classifying the cooled mixture to obtain the toner.

These and other objects, features and advantages of the present invention will become more apparent upon a consideration of the following description concluding

with specific examples and comparative examples taken in conjunction with the accompanying drawing.

#### BRIEF DESCRIPTION OF THE DRAWING

The sole FIGURE in the drawing shows a chromatogram of gel permeation chromatography of the resin obtained in Example 1.

#### DETAILED DESCRIPTION OF THE INVENTION

Critical features of the present invention for accomplishing the above objects are that the binder resin has at least three peaks or shoulders in its molecular weight distribution curve, that the molecular weight  $Ma$  of a peak or shoulder giving the smallest molecular weight is within the range of 2,000 to 80,000 and that the molecular weight  $Mc$  of a peak or shoulder giving the largest molecular weight and the above mentioned  $Ma$  gives a ratio  $Mc/Ma$  of 150 or larger.

According to a preferred embodiment of the present invention, at least one of the above-mentioned at least three peaks or shoulders is present in each of the three regions, namely a molecular weight region A of  $2 \times 10^3$  to  $8 \times 10^4$ , molecular weight region B of  $3 \times 10^5$  to  $10^6$ , and molecular weight region C of  $3 \times 10^6$  or larger; and, when the heights of the peaks or shoulders in the three regions are denoted by  $Ha$ ,  $Hb$  and  $Hc$ , respectively, these values satisfy the proportional relationship of  $Ha:Hb:Hc = 1:0.2-1.0:0.1-0.6$ .

Among the components of the binder resin respectively present in the regions A, B and C, the component in the region B provides basic properties of a heat-fixable dry-system developer. The component in the region A is critical in improving the characteristic of fixation to a transfer material under heat and pressure. Further, the component in the region C functions to remarkably improve the anti-offset property of a toner against rollers during hot roller fixation and to improve the pealability or releasability from the rollers of a transfer material such as paper after fixation, and also plays an essential role in the durability in successive copying and adaptability to a variety of environments of a toner.

Furthermore, the ratio  $Mc/Ma$  between the molecular weight  $Mc$  giving the peak in the region C and the molecular weight  $Ma$  giving the peak in the region A, and the ratios among the heights  $Ha$ ,  $Hb$  and  $Hc$  of the peaks respectively in the three regions, are also very important factors for further improving fixability under heat and pressure as well as anti-offset characteristic during hot-roller fixation and satisfying the durability in successive copying and adaptability to various environments.

The height  $H$  used herein of a peak or shoulder refers to a length of a perpendicular to the base line from each peak or shoulder on a chromatogram chart of GPC. For the case of a shoulder, the perpendicular from the point of flection of the shoulder to the base line gives the height.

A proposal for giving a toner with improved fixability by mixing a plurality of component binder resins having different molecular weight ranges has been made, but satisfactory binder resins have not yet been obtained. More specifically, the thus provided binder resin has not fully dissolved the problem of fixing performance or anti-offset characteristic during heat fixation by means of hot rollers but still involves some problem in respect of durability.

The Japanese Patent Laid-Open Application No. 82258/1983 discloses examples of binder resins having three peaks in the molecular weight distribution, but it is not always sufficient for a binder resin to have three peaks. For example, when the  $Ma/Mc$  values are calculated with respect to the binder resins having three peaks disclosed in the above-mentioned Laid-Open Application in the light of the present invention, they are all within the range of 20-90. Thus, the difference between the  $Ma$  and  $Mc$  is not sufficient, and a toner containing the resin can cause off-setting when the hot roller temperature is around 200°C. In contrast thereto, the binder resin of the present invention is characterized by having an  $Mc/Ma$  ratio of 150 or larger and having a sufficiently large difference between the  $Ma$  and  $Mc$ . As described hereinbefore, the  $Ma$  value relates to the fixing performance onto a transfer material or the minimum fixable temperature of a toner, and the  $Mc$  value relates to the high-temperature anti-offset characteristic onto hot rollers or the off-set initiating temperature of a toner. Accordingly, it is desired to decrease  $Ma$  so as to secure a lower fixing temperature and at the same time to increase  $Mc$  so as not to impair the anti-offset characteristic, whereby the fixation temperature range (i.e., temperature range applicable for fixation) is enlarged. From this point of view, the  $Mc/Ma$  ratio of 20 to 90 does not give a wide fixation temperature range but results in a toner with considerable room for improvement in various fixation characteristics. In contrast therewith, the  $Mc/Ma$  ratio of 150 or larger gives a toner with a sufficiently wide fixation temperature range and showing good overall fixation characteristics on hot roller fixation, which is sufficiently fixable with a relatively small amount of heat, almost free from off-setting onto hot rollers and capable of effecting smooth paper discharge from rollers. Further, the  $Mc$  value thus enlarged is also effective in improving the durability of a toner.

The peak in the region A of the binder resin according to the invention is a principal factor for determining the fixability under heat and pressure, in other words, the minimum fixable temperature on hot roller fixation. If the peak has a smaller molecular weight, the fixation temperature can be lowered which is desirable in respect of fixability. On the other hand, a smaller molecular weight for the peak in the region A results in poorer anti-offset characteristic onto rollers and poorer transfer paper-releasability during fixation. The molecular weight  $Ma$  for the peak in the region A is in the range of 2,000 to 80,000, preferably in the range of 2,000 to 40,000, and more preferably in the range of 5,000 to 20,000.

The peak in the high molecular weight region C is critical to the anti-offset characteristic and gives better overall characteristics in combination with and in compensation for each other with the peak in the region A as described above. In other words, a better fixability and a better anti-offset characteristic are harmonized in combination by the balance between the components of the regions A and C. For this purpose, the ratio  $Mc/Ma$  between molecular weights for the peaks in the respective regions is required to be 150 or larger and is further preferred to satisfy the following relationship:

$$-2.5 \times 10^2 \times Ma + 5.5 \times 10^6 \geq Mc \geq -5 \times 10^2 \times Ma + 1.5 \times 10^7$$

It is also to be noted that the ratios among the heights of the respective peaks in the regions A, B and C play an important role in improving the problems encountered with the conventional binder resins. If the molecular weights Ma, Mb and Mc of the peaks are referred to as qualitative factors, the heights Ha, Hb and Hc are quantitative factors, and the balance among Ha, Hb and Hc has a critical influence on the heat fixing characteristics and durability of a toner and the easiness of operation such as kneading under heat, pulverization, etc., for 10 production of a toner.

The ratios among Ha:Hb:Hc are preferably 1:0.2-1.0:0.1-0.6 and more preferably 1:0.4-0.8:0.15-0.4. Too large Ha relative to Hb results in offsetting of a toner onto rollers and poor releasability of transfer paper, increase in agglomeration tendency and increased liability of deterioration during successive use of a toner. To the contrary, too small Ha relative to Hb results in poor fixability of a toner. Too large Hc relative to Hb results in poor fluidity of a toner on heating and fails to realize sufficient fixation. Further, the pulverizability is noticeably lowered thereby, so that the toner material containing the binder cannot be effectively pulverized into a desirable particle size for a toner on a commercial scale. To the contrary, too small Hc 25 relative to Hb fails to ensure sufficient anti-offset characteristic and releasability of transfer paper during fixation.

A molecular weight in the region C, i.e., a molecular weight above three million cannot be measured accurately according to the gel permeation chromatography in the present state. Accordingly, the molecular weight values in this region used in the present invention have been obtained by extrapolation of a calibration curve 35 obtained based on standard samples in the molecular weight range of upto around two million where accurate measurement is possible.

The binder resin for a toner according to the present invention having the above mentioned molecular weight distribution may be prepared by synthesis while adjusting the conditions therefor. Alternatively, the binder resin may be prepared by mixing a plurality of polymers, e.g., a polymer (A) having a peak or shoulder in the molecular weight range of  $10^3$  to  $8 \times 10^4$ , a polymer (B) having a peak or shoulder in the molecular weight range of  $3 \times 10^5$  to  $10^6$ , and a polymer (C) having a peak or shoulder in the molecular weight range of  $3 \times 10^6$  or larger. When a plurality of polymers are mixed, the mixing ratios among the polymers A, B and C should desirably be as follows with the polymer B as the base polymer. The mixing weight ratio of the polymer A/the polymer B is desirably in the range of 5/1 to 1/1. The weight ratio of the polymer C/the polymer B is desirably in the range of 1:1 to 1/5. If the polymer A is too much relative to the polymer B, offsetting onto 55 rollers occurs and releasability of transfer paper is deteriorated. To the contrary, if the polymer is too little, sufficient fixability of a toner cannot be obtained. If the polymer C is too much relative to the polymer B, fluidity of a toner on heating becomes worse and sufficient fixation cannot be effected. Further, the pulverization becomes noticeably difficult and a particle size adapted for a dry system developer cannot be effectively obtained by pulverization on a commercial scale. More specifically, an economically feasible range of productivity cannot be accomplished by an ordinary pulverizing means. To the contrary, if the polymer C is too little, sufficient releasability or anti-offset characteristic

can not be ensured. The polymers A, B and C need not necessarily have the same composition but should desirably comprise the same monomer as the principal component, respectively.

5 The number of the peaks or shoulders contained in the chromatograph of the binder resin is not necessarily three but may be four or more. In the latter case, it is sufficient for three peaks or shoulders among them to satisfy the above mentioned requirements of the present invention.

As described hereinbefore, the binder resin of the present invention has a peak respectively in the three molecular weight regions A, B and C, and the peak molecular weights Ma and Mc satisfy the relationships of  $Ma = 2,000-80,000$  and  $Mc/Ma \geq 150$ . Herein, the chromatogram giving the molecular weight distribution is somewhat changed according to a measurement method adopted. In the present invention, the following method has been adopted for giving a chromatogram and a molecular weight of a resin, based on which the values for characterizing the inventions have been defined. Of course, other gel permeation chromatographic methods can be adopted for evaluation of a resin as far as they give substantially equivalent measurement values.

A chromatograph LC-3A provided with columns HSG 60, HSG 40 and HSG 15 arranged in series (available from Shimazu Seisakusho K. K.) is used at an over temperature of 40° C. While a solvent THF (tetrahydrofuran) is passed at a rate of 1.7 ml/min. under a fluid pressure of 90 kg/cm<sup>2</sup>, 500  $\mu$ l of a sample solution in THF at a concentration of 0.4 g/dl is injected. The sample solution is prepared by dissolving a sample resin in THF and passing the solution through a membrane filter (TM-2P 0.45  $\mu$ m, produced by Toyo Roshi K. K.) and is injected one hour after the dissolution.

For the measurement of the molecular weight of a sample, a calibration curve is prepared by using 6 samples (Molecular Weights: 2,000,000; 600,000; 233,000; 50,000; 17,500; and 2,200; produced by Pressure Chemical Co.). Among the 6 standard samples, 3 samples (M.W.: 2,000,000; 233,000 and 17,500) are mixed in equal proportions and are made into a THF solution at a concentration of 0.4 g/dl, which is injected in a volume of 500  $\mu$ l, 24 hours after the dissolution. Separately, the other 3 standard samples (M.W.: 600,000; 50,000 and 2,200) and also mixed in equal amounts into a 0.4 g/dl THF solution, which is then likewise injected. In the Examples and Comparative Examples described herein-after, the analyzer used was a differential refractometer (RID-2A, produced by Shimazu Seisakusho K.K.).

The binder resin according to the invention can be prepared in the following processes.

Ordinary polymerization processes give a molecular weight distribution with a single peak. Accordingly, the following specific processes may preferably be adopted in order to produce the binder resin of the present invention. Those processes include a process wherein polymerization is carried out at stepwise different temperatures; a process wherein monomer mixtures containing different concentrations of initiators or chain transfer agents are intermittently added to a system to be polymerized; and a process wherein a crosslinking agent is intentionally added to a monomer mixture system to be polymerized. A process wherein polymerization conditions are controlled with the use of a crosslinking agent is a particularly preferred for the purpose of obtaining the resin of the present invention.

While these processes can be practiced by solution polymerization, suspension polymerization, emulsion polymerization, etc., the solution polymerization process is especially preferred for the reason that the molecular weight distribution can be controlled more easily. As another method, the resin having the desired molecular weight distribution can be obtained by mixing at a molecular level a plurality of resins including a resin of a relatively low molecular weight and a resin of a high molecular weight. More specifically, this is accomplished by a process wherein a plurality of resins of different molecular weights are dissolved in a solvent and, after sufficient mixing, the solvent is removed or by a process of melting such a plurality of resins under heating and blending the melted resins. In order to accomplish the objects of the present invention, it is preferred to obtain a resin having the ultimately objective molecular weight distribution in the polymerization stage.

A preferred process for producing the resin according to the present invention is as follows.

A mixture of vinyl monomers containing a crosslinking monomer is subjected to solution polymerization in the presence of an organic solvent capable of dissolving the copolymer of the vinyl monomer mixture and a polymerization initiator having a 10 hour-half life temperature, i.e., a temperature giving a half life of 10 hours, of 100° C. or higher. The solution polymerization is carried out at a temperature of 0°-40° C. higher than the 10 hour-half life temperature. Thus, a vinyl copolymer having the molecular weight distribution according to the invention is obtained.

The binder resin of the invention can be constituted by various components as far as they can constitute a toner resin and they can give the above mentioned molecular weight distribution. Especially, vinyl monomers are preferred to give vinyl copolymers.

Examples of the vinyl monomers applicable to the present invention include: styrene and its derivatives such as styrene,  $\alpha$ -methylstyrene, and p-chlorostyrene; monocarboxylic acids and their derivatives such as acrylic acid, methyl acrylate, ethyl acrylate, butyl acrylate, dodecyl acrylate, octyl acrylate, phenyl acrylate, methacrylic acid, methyl methacrylate, ethyl methacrylate, butyl methacrylate, octyl methacrylate, acrylonitrile, and acrylamide; dicarboxylic acids having a double bond and their derivatives such as maleic acid, monobutyl maleate, dibutyl maleate, monomethyl maleate and dimethyl maleate; vinyl esters such as vinyl chloride, vinyl acetate, and vinyl benzoate; vinyl ketones such as vinyl methyl ketone and vinyl ethyl ketone; and vinyl ethers such as vinyl methyl ether, vinyl ethyl ether and vinyl isobutyl ether. These vinyl monomers are used alone or in a mixture. The binder resin of the invention may preferably be constituted by a styrene copolymer.

Such a vinyl copolymer giving the above mentioned chromatogram is preferred to constitute 60 % by weight or more, particularly 70 % by weight or more of the toner binder resin.

Selection of initiators, solvents and reaction conditions is important for obtaining the objective resin of the invention. Examples of the applicable initiators include organic peroxides such as, 1,1-(*t*-butylperoxy)-3,3,5-trimethylcyclohexane, n-butyl-4,4-di(*t*-butylperoxy)-valerate, dicumyl peroxide,  $\alpha,\alpha'$ -bis(*t*-butylperoxydiisopropyl)benzene, *t*-butylperoxycumene and di-*t*-butylperoxide; and azo and diazo compounds such as

diazoaminoazobenzene. Particularly useful class of polymerization initiators are those having a 10 hour-half life temperature of 100° C. or above as mentioned hereinbefore. Especially, di-*t*-butyl peroxide is effective. In this instance, the polymerization temperature is preferably selected at a temperature higher than the 10 hour-half life temperature by 0°-40° C. and accordingly a solvent adapted to the temperature is preferably selected.

Generally, the molecular weight  $M_a$  decreases, as the amount of the initiator increases, as the concentration of the monomer in the reaction system is decreased relative to the solvent, and as the reaction time is prolonged. Further, as the concentration of the crosslinking monomer increases, the molecular weight  $M_c$  increases and the height  $H_c$  increases.

The copolymer should preferably be crosslinked to some extent to give better anti-offset characteristic. There are various methods of causing some degree of crosslinking. For example, the above mentioned method of effecting copolymerization in the presence of a crosslinking monomer to obtain a vinyl copolymer is an effective method.

The crosslinking monomer may chiefly be compounds having two or more polymerizable double bonds. Examples of such compounds include: aromatic divinyl compounds such as divinylbenzene and divinyl-naphthalene; carboxilic acid esters having two double bonds such as ethylene glycol diacrylate, ethylene glycol dimethacrylate, and 1,3-butanediol dimethacrylate; divinyl compounds such as divinylaniline, divinyl ether, divinyl sulfide and divinyl sulfone; and compounds having three or more vinyl groups. Among these, divinylbenzene is particularly useful.

Such a crosslinking monomer should preferably be contained in 0.2 to 5 parts by weight, particularly 0.8 to 2.5 parts by weight, in 100 parts by weight of the vinyl monomer mixture.

The binder resin of the invention should preferably have a softening point according to the ring and ball test of the order of 100° to 150° C., while it varies to some extent depending on the monomers and composition thereof. The glass transition temperature may preferably be in the range of 40° to 80° C., and, more preferably, 50° to 60° C. If the softening point is below 100° C., the toner causes filming to soil the photosensitive member or readily deteriorates during successive copying. If it exceeds 150° C., fixation efficiency is lowered due to increase in fixable temperature, and the pulverization efficiency is also decreased. If the glass transition temperature is lower than 40° C., thermal agglomeration or caking of the toner can readily occur during storage of the toner, so that agglomeration trouble can occur also in a copying machine. To the contrary, if the glass transition temperature exceeds 80° C., the heat fixation efficiency becomes worse.

The binder resin of the present invention should preferably have an M.I. (melt index) in the range of 0.25 to 5 under the conditions of 125° C. and 2160 g and more preferably in the range of 1.2 to 4. An M.I. of below 0.5 leads to increase in fixation temperature and decrease in fixation efficiency of the toner. If the M.I. is larger than 5, offsetting onto rollers readily occurs during high temperature fixation.

The softening point (S.P.) of the ring and ball method is based on the values obtained according to JIS K 2531 and the melt index (M.I.) according to JIS K 7210. The glass transition temperature (Tg) is based on the values

obtained by means of a differential thermal analyzer DTA-30M (available from Shimazu Seisakusho K. K.) under the conditions of a temperature raising rate of 15° C./min. and a sample weight of 10 to 15 mg.

The toner for a developer of the invention can contain other resinous compounds in addition to the above mentioned binder resin according to the invention in a proportion less than the latter. Examples of such resinous compounds include silicone resin, polyester, polyurethane, polyamide, epoxy resin, polyvinylbutyral, rosin, modified rosin, terpene resin, aliphatic or alicyclic hydrocarbon resin, aromatic petroleum resin, chlorinated paraffin, and paraffin wax.

When a magnetic toner is produced, magnetic particles are contained in the toner. The magnetic particles may be a material which shows magnetism by itself or which is magnetizable. Examples of such materials include metals such as iron, manganese, nickel, cobalt and chromium, magnetite, hematite, various ferrites, manganese alloys, and other ferromagnetic alloys. The magnetic particles may be obtained by rendering these materials into fine particles having an average particle size of about 0.05 to 5 $\mu$ , more preferably 0.1 to 2 $\mu$ . A magnetic toner should preferably contain such magnetic particles in a proportion of 1.5 to 70 %, particularly 25 to 45 % of the total toner weight.

The toner of the present invention can further contain a colorant, a charge controller agent, or a flowability improver. Examples of such materials include carbon black, iron black, graphite, nigrosine, metal complexes of monoazo dyes, Hansa Yellow, Benzidine Yellow, Quinacridone and various lake pigments.

A flowability improver such as hydrophobic colloidal silica may be externally mixed with the toner particles. The flowability improver may be added in an amount of 0.05 to 5 wt. %, preferably 0.1 to 2 wt. %, of the toner.

The toner produced from the above mentioned binder resin, magnetic particles colorant, charge controller agent, etc., is highly resistant to a load applied in a developing apparatus and is very seldom deteriorated due to crushing during durability test. On the other hand, it is desirable to add a small amount of an olefinic homopolymer or copolymer having a melt viscosity at 140° C. of 10 to 10<sup>6</sup> cps, more preferably 10<sup>2</sup> to 10<sup>5</sup> cps, in order to prevent abrasion of or damage to the surface of a photosensitive member, a cleaning member, the surface of a developing sleeve, carrier particles, etc. When such an additive is externally added to the toner particles, a weight ratio thereof to the toner can vary to change developing characteristics during repetitive use. For this reason, the additive is preferably incorporated in the toner. If the olefinic polymer is contained in the developer powder in a proportion of 0.5 to 5 wt. %, the dispersibility and compatibility of pigment or magnetic particles with respect to the toner are improved, and good effects for the surface of a photosensitive member, a cleaning member, etc., are attained. Examples of the olefinic homopolymer or copolymer used for this purpose include polyethylene, polypropylene, ethylene-propylene copolymer, ethylene-vinyl acetate copolymer, ethylene-ethyl acrylate copolymer and ionomer resin having a polyethylene base structure. When an olefinic copolymer is used, the copolymer should preferably contain 50 mol. % or more, more preferably 60 mol. % or more of olefin monomer units.

The melt viscosities have been measured according to the Brookfield method and with a Brookfield viscometer provided with an adaptor for a small amount sample.

An electrophotographic process using the toner of the present invention will be explained hereinbelow.

There are various methods for developing electric latent images with a toner, such as the magnetic brush method as mentioned above, the cascade method, the powder cloud method, a method wherein an electroconductive magnetic toner is used as disclosed in U.S. Pat. No. 3,909,258, and a method wherein a high resistivity magnetic toner is used as disclosed in Japanese Patent Laid-Open Application No. 31136/1978. A developer obtained by using the resin of the present invention is also suitable for a developing method using a so-called one-component developer containing magnetic particles.

In a step of transferring a developed image to a part to be transfer-printed, various systems may be adopted such as the corona transfer system, the bias transfer system, an electrostatic transfer system such as a system using an electroconductive roller, and a system using a magnetic field for the transfer.

Residual toner on the photosensitive layer or insulating layer may be removed by the blade cleaning system or the fur brush cleaning system.

Powder image on a transfer-printed member should be fixed, for example by the heat fixing method, the solvent fixing method, the flash fixing method, or the laminate fixing method. In order to fully exhibit the characteristics of the toner according to the invention, the hot roller fixing method is preferably adopted.

As described in detail hereinabove, according to the present invention, there is provided a resin for a toner having at least three peaks or shoulders in its molecular weight distribution curve and a specific molecular weight difference between two peaks or shoulders respectively giving the largest and smallest molecular weights. By using the toner, there is further obtained a toner which is particularly excellent in harmonization of fixability, anti-offset characteristic and durability.

The present invention will be described more specifically hereinbelow by referring to the examples and comparative examples, wherein "parts" means "parts by weight".

#### EXAMPLE 1

|    | Mixture             | Quantity           |
|----|---------------------|--------------------|
| 50 | Styrene             | 414 g (69 parts)   |
|    | n-Butyl acrylate    | 141 g (23.5 parts) |
|    | Monobutyl maleate   | 36 g (6 parts)     |
|    | Divinylbenzene      | 8.4 g (1.4 parts)  |
|    | Di-t-butyl peroxide | 6.0 g (1.0 parts)  |

55  
60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
770  
771  
772  
773  
774  
775  
776  
777  
778  
779  
780  
781  
782  
783  
784  
785  
786  
787  
788  
789  
790  
791  
792  
793  
794  
795  
796  
797  
798  
799  
800  
801  
802  
803  
804  
805  
806  
807  
808  
809  
8010  
8011  
8012  
8013  
8014  
8015  
8016  
8017  
8018  
8019  
8020  
8021  
8022  
8023  
8024  
8025  
8026  
8027  
8028  
8029  
8030  
8031  
8032  
8033  
8034  
8035  
8036  
8037  
8038  
8039  
8040  
8041  
8042  
8043  
8044  
8045  
8046  
8047  
8048  
8049  
8050  
8051  
8052  
8053  
8054  
8055  
8056  
8057  
8058  
8059  
8060  
8061  
8062  
8063  
8064  
8065  
8066  
8067  
8068  
8069  
8070  
8071  
8072  
8073  
8074  
8075  
8076  
8077  
8078  
8079  
8080  
8081  
8082  
8083  
8084  
8085  
8086  
8087  
8088  
8089  
8090  
8091  
8092  
8093  
8094  
8095  
8096  
8097  
8098  
8099  
80100  
80101  
80102  
80103  
80104  
80105  
80106  
80107  
80108  
80109  
80110  
80111  
80112  
80113  
80114  
80115  
80116  
80117  
80118  
80119  
80120  
80121  
80122  
80123  
80124  
80125  
80126  
80127  
80128  
80129  
80130  
80131  
80132  
80133  
80134  
80135  
80136  
80137  
80138  
80139  
80140  
80141  
80142  
80143  
80144  
80145  
80146  
80147  
80148  
80149  
80150  
80151  
80152  
80153  
80154  
80155  
80156  
80157  
80158  
80159  
80160  
80161  
80162  
80163  
80164  
80165  
80166  
80167  
80168  
80169  
80170  
80171  
80172  
80173  
80174  
80175  
80176  
80177  
80178  
80179  
80180  
80181  
80182  
80183  
80184  
80185  
80186  
80187  
80188  
80189  
80190  
80191  
80192  
80193  
80194  
80195  
80196  
80197  
80198  
80199  
80200  
80201  
80202  
80203  
80204  
80205  
80206  
80207  
80208  
80209  
80210  
80211  
80212  
80213  
80214  
80215  
80216  
80217  
80218  
80219  
80220  
80221  
80222  
80223  
80224  
80225  
80226  
80227  
80228  
80229  
80230  
80231  
80232  
80233  
80234  
80235  
80236  
80237  
80238  
80239  
80240  
80241  
80242  
80243  
80244  
80245  
80246  
80247  
80248  
80249  
80250  
80251  
80252  
80253  
80254  
80255  
80256  
80257  
80258  
80259  
80260  
80261  
80262  
80263  
80264  
80265  
80266  
80267  
80268  
80269  
80270  
80271  
80272  
80273  
80274  
80275  
80276  
80277  
80278  
80279  
80280  
80281  
80282  
80283  
80284  
80285  
80286  
80287  
80288  
80289  
80290  
80291  
80292  
80293  
80294  
80295  
80296  
80297  
80298  
80299  
80300  
80301  
80302  
80303  
80304  
80305  
80306  
80307  
80308  
80309  
80310  
80311  
80312  
80313  
80314  
80315  
80316  
80317  
80318  
80319  
80320  
80321  
80322  
80323  
80324  
80325  
80326  
80327  
80328  
80329  
80330  
80331  
80332  
80333  
80334  
80335  
80336  
80337  
80338  
80339  
80340  
80341  
80342  
80343  
80344  
80345  
80346  
80347  
80348  
80349  
80350  
80351  
80352  
80353  
80354  
80355  
80356  
80357  
80358  
80359  
80360  
80361  
80362  
80363  
80364  
80365  
80366  
80367  
80368  
80369  
80370  
80371  
80372  
80373  
80374  
80375  
80376  
80377  
80378  
80379  
80380  
80381  
80382  
80383  
80384  
80385  
80386  
80387  
80388  
80389  
80390  
80391  
80392  
80393  
80394  
80395  
80396  
80397  
80398  
80399  
80400  
80401  
80402  
80403  
80404  
80405  
80406  
80407  
80408  
80409  
80410  
80411  
80412  
80413  
80414  
80415  
80416  
80417  
80418  
80419  
80420  
80421  
80422  
80423  
80424  
80425  
80426  
80427  
80428  
80429  
80430  
80431  
80432  
80433  
80434  
80435  
80436  
80437  
80438  
80439  
80440  
80441  
80442  
80443  
80444  
80445  
80446  
80447  
80448  
80449  
80450  
80451  
80452  
80453  
80454  
80455  
80456  
80457  
80458  
80459  
80460  
80461  
80462  
80463  
80464  
80465  
80466  
80467  
80468  
80469  
80470  
80471  
80472  
80473  
80474  
80475  
80476  
80477  
80478  
80479  
80480  
80481  
80482  
80483  
80484  
80485  
80486  
80487  
80488  
80489  
80490  
80491  
80492  
80493  
80494  
80495  
80496  
80497  
80498  
80499  
80500  
80501  
80502  
80503  
80504  
80505  
80506  
80507  
80508  
80509  
80510  
80511  
80512  
80513  
80514  
80515  
80516  
80517  
80518  
80519  
80520  
80521  
80522  
80523  
80524  
80525  
80526  
80527  
80528  
80529  
80530  
80531  
80532  
80533  
80534  
80535  
80536  
80537  
80538  
80539  
80540  
80541  
80542  
80543  
80544  
80545  
80546  
80547  
80548  
80549  
80550  
80551  
80552  
80553  
80554  
80555  
80556  
80557  
80558  
80559  
80560  
80561  
80562  
80563  
80564  
80565  
80566  
80567  
80568  
80569  
80570  
80571  
80572  
80573  
80574  
80575  
80576  
80577  
80578  
80579  
80580  
80581  
80582  
80583  
80584  
80585  
80586  
80587  
80588  
80589  
80590  
80591  
80592  
80593  
80594  
80595  
80596  
80597  
80598  
80599  
80600  
80601  
80602  
80603  
80604  
80605  
80606  
80607  
80608  
80609  
80610  
80611  
80612  
80613  
80614  
80615  
80616  
80617  
80618  
80619  
80620  
80621  
80622  
80623  
80624  
80625  
80626  
80627  
80628  
80629  
80630  
80631  
80632  
80633  
80634  
80635  
80636  
80637  
80638  
80639  
80640  
80641  
80642  
80643  
80644  
80645  
80646  
80647  
80648  
80649  
80650  
80651  
80652  
80653  
80654  
80655  
80656  
80657  
80658  
80659  
80660  
80661  
80662  
80663  
80664  
80665  
80666  
80667  
80668  
80669  
80670  
80671  
80672  
80673  
80674  
80675  
80676  
80677  
80678  
80679  
80680  
80681  
80682  
80683  
80684  
80685  
80686  
80687  
80688  
80689  
80690  
80691  
80692  
80693  
80694  
80695  
80696  
80697  
80698  
80699  
80700  
80701  
80702  
80703  
80704  
80705  
80706  
80707  
80708  
80709  
80710  
80711  
80712  
80713  
80714  
80715  
80716  
80717  
80718  
80719  
80720  
80721  
80722  
80723  
80724  
80725  
80726  
80727  
80728  
80729  
80730  
80731  
80732  
80733  
80734  
80735  
80736  
80737  
80738  
80739  
80740  
80741  
80742  
80743  
80744  
80745  
80746  
80747  
80748  
80749  
80750  
80751  
80752  
80753  
80754  
80755  
80756  
80757  
80758  
80759  
80760  
80761  
80762  
80763  
80764  
80

in the attached drawing and had peaks at molecular weights of 13,000; 870,000; and 4,500,000, indicating an  $Mc/Ma$  of 346 and  $Ha/Hb/Hc$  or 1/0.5/0.2. The polymer obtained also had a  $T_g$  of 57° C. and M.I. of 2.3.

### EXAMPLE 2

Polymerization was conducted in the same manner as in Example 1 except that the n-butyl acrylate was replaced by 2-ethylhexyl acrylate and the following mixture was used.

| Mixture               | Quantity           |
|-----------------------|--------------------|
| Styrene               | 435 g (75.7 parts) |
| 2-Ethylhexyl acrylate | 102 g (17 parts)   |
| Monobutyl maleate     | 36 g (6 parts)     |
| Divinylbenzene        | 8.4 g (1.4 parts)  |
| Di-t-butyl peroxide   | 6.0 g (1.0 parts)  |

The properties of the copolymer obtained are summarized in Table 1B appearing hereinafter.

### EXAMPLES 3-7, COMPARATIVE EXAMPLES 1-3

The compositions of monomer mixtures and polymerization conditions of these examples are summarized in the following Table 1A and the results in Table 1B, together with those of Examples 1 and 2. The operation procedure of these examples was substantially the same as that of Example 1 explained above.

TABLE 1A

| Example              | List of Examples (Synthesis) |              |           |               |             |                |                       |                  |
|----------------------|------------------------------|--------------|-----------|---------------|-------------|----------------|-----------------------|------------------|
|                      | Monomers (parts)             |              |           |               | Initiator   | Solvent        | Temperature           | Time             |
|                      | 1                            | 2            | 3         | 4             |             |                |                       |                  |
| 1                    | Styrene<br>(69)              | BA<br>(23.5) | MB<br>(6) | DVB<br>(1.4)  | DBPO<br>1.0 | Xylene<br>70   | Reflux<br>temperature | 3 hr.<br>20 min. |
| 2                    | Styrene<br>(75.5)            | 2EHA<br>(17) | MB<br>(6) | DVB<br>(1.4)  | DBPO<br>1.0 | Xylene<br>70   | Reflux<br>temperature | 3 hr.<br>20 min. |
| 3                    | Styrene<br>(70)              | BA<br>(23.5) | MB<br>(6) | DVB<br>(0.55) | DBPO<br>0.5 | Xylene<br>50   | Reflux<br>temperature | 3 hr.<br>20 min. |
| 4                    | Styrene<br>(76.5)            | 2EHA<br>(17) | MB<br>(6) | DVB<br>(0.55) | DBPO<br>0.5 | Xylene<br>50   | Reflux<br>temperature | 3 hr.<br>20 min. |
| 5                    | Styrene<br>(69.5)            | BA<br>(20)   | MB<br>(6) | DVB<br>(4.5)  | DBPO<br>4   | Xylene<br>100  | Reflux<br>temperature | 4 hr.<br>20 min. |
| 6                    | Styrene<br>(74.5)            | 2EHA<br>(15) | MB<br>(6) | DVB<br>(4.5)  | DBPO<br>4   | Xylene<br>100  | Reflux<br>temperature | 4 hr.<br>20 min. |
| 7                    | Styrene<br>(71.5)            | LMA<br>(18)  | MB<br>(6) | DVB<br>(4.3)  | DBPO<br>4   | Xylene<br>100  | Reflux<br>temperature | 4 hr.<br>20 min. |
| Comparative Examples |                              |              |           |               |             |                |                       |                  |
| 1                    | Styrene<br>(70)              | BA<br>(23.5) | MB<br>(6) | DVB<br>(0.15) | DBPO<br>2   | Toulene<br>100 | Reflux<br>temperature | 3 hr.<br>20 min. |
| 2                    | Styrene<br>(70)              | BA<br>(23.5) | MB<br>(6) | DVB<br>(0.48) | DBPO<br>0.5 | Xylene<br>50   | Reflux<br>temperature | 3 hr.<br>20 min. |
| 3                    | Styrene<br>(70)              | BA<br>(20)   | MB<br>(6) | DVB<br>(3.7)  | DBPO<br>4   | Xylene<br>100  | Reflux<br>temperature | 4 hr.<br>20 min. |

BA — butyl acrylate

2EHA — 2-ethylhexyl acrylate

LMA — lauryl methacrylate

MB — monobutyl maleate

DVB — divinylbenzene

DBPO — di-t-butylperoxide

TABLE 1B

| Example             | Tg     | MI  | Peak molecular weight ( $\times 10^3$ ) |     |      | $Mc/Ma$ | $Ha/Hb/Hc$ |
|---------------------|--------|-----|-----------------------------------------|-----|------|---------|------------|
|                     |        |     | Ma                                      | Mb  | Mc   |         |            |
| 1                   | 57° C. | 2.3 | 13                                      | 870 | 4500 | 346     | 1/0.5/0.2  |
| 2                   | 56     | 2.2 | 14                                      | 800 | 4300 | 307     | 1/0.5/0.2  |
| 3                   | 65     | 1.4 | 23                                      | 950 | 4100 | 178     | 1/0.8/0.15 |
| 4                   | 64     | 1.3 | 25                                      | 930 | 3900 | 156     | 1/0.7/0.2  |
| 5                   | 62     | 2.5 | 9                                       | 700 | 6500 | 722     | 1/0.4/0.6  |
| 6                   | 61     | 3.0 | 9                                       | 720 | 6800 | 756     | 1/0.4/0.5  |
| 7                   | 62     | 2.5 | 10                                      | 690 | 7000 | 700     | 1/0.4/0.6  |
| Comparative Example |        |     |                                         |     |      |         |            |
| 15                  | 64     | 0.7 | 52                                      | 610 | 2100 | 40      | 1/0.6/0.05 |
| 2                   | 63     | 2.5 | 31                                      | 630 | —    | —       | 1/0.5/—    |
| 3                   | 59     | 7.5 | 9                                       | 600 | —    | —       | 1/0.7/—    |

### EXAMPLES 8-11, COMPARATIVE EXAMPLES 4-5

Resins according to the present invention and comparative resins were respectively obtained by uniformly mixing a plurality of polymers as shown in the following Table 2A.

More specifically, in each example, a plurality of polymers were respectively dissolved in toluene and the resultant solutions were uniformly mixed so as to effect mixing at molecular level. Then, the solvent toluene was removed by reduced pressure distillation to leave a resin mixture.

The measured properties of the resultant resin mixtures are shown in Table 2B.

TABLE 2A

| Example | List of Examples (Mixing) |  |  | Monomer mole ratio | Average M.W. ( $\times 10^4$ ) | Weight % |
|---------|---------------------------|--|--|--------------------|--------------------------------|----------|
|         | Polymer species           |  |  |                    |                                |          |
|         |                           |  |  |                    |                                |          |

TABLE 2A-continued

|                     |                         | List of Examples (Mixing) |                                |          |
|---------------------|-------------------------|---------------------------|--------------------------------|----------|
|                     | Polymer species         | Monomer mole ratio        | Average M.W. ( $\times 10^4$ ) | Weight % |
| 8                   | Styrene-BA copolymer    | 72/28                     | 6.2                            | 65       |
|                     | Styrene-BA copolymer    | 72/28                     | 60                             | 25       |
|                     | Styrene-2EHA copolymer  | 75/25                     | 220                            | 10       |
| 9                   | Styrene-BA copolymer    | 70/30                     | 1.8                            | 60       |
|                     | Styrene-BA copolymer    | 72/28                     | 65                             | 32       |
|                     | Styrene-BA copolymer    | 70/30                     | 260                            | 8        |
| 10                  | Styrene-BA copolymer    | 70/30                     | 2.4                            | 50       |
|                     | Styrene-BA-MB copolymer | 70/25/5 (two peaks)       | 140                            | 50       |
| 11                  | Styrene-BA-MA copolymer | 70/24/6 (two peaks)       | 120                            | 88       |
|                     | Styrene-BA copolymer    | 80/20                     | 360                            | 12       |
| Comparative Example |                         |                           |                                |          |
| 4                   | Styrene-BA copolymer    | 72/28                     | 2.5                            | 75       |
|                     | Styrene-BA copolymer    | 65/35                     | 50                             | 25       |
|                     | Styrene-BA copolymer    | 70/30                     | 8                              | 65       |
| 6                   | Styrene-BA copolymer    | 70/30                     | 30                             | 25       |
|                     | Styrene-BA copolymer    | 65/35                     | 115                            | 10       |
|                     | Styrene-BA copolymer    | 65/35                     | 1.25                           | 60       |
|                     | Styrene-BA copolymer    | 65/35                     | 20.5                           | 30       |
|                     | Styrene-BA copolymer    | 65/35                     | 115                            | 10       |

BA — butyl acrylate

MB — monobutyl maleate

2EHA — 2-ethylhexyl acrylate

TABLE 2B

| Example             | Ma   | Mb  | Mc   | Mc/Ma | Ha | Hb   | Hc/Tg/MI    |
|---------------------|------|-----|------|-------|----|------|-------------|
| 8                   | 12   | 410 | 3200 | 267   | 1  | 0.4  | 0.17/57/1.6 |
| 9                   | 14   | 520 | 3900 | 279   | 1  | 0.6  | 0.21/59/2.1 |
| 10                  | 12   | 500 | 4500 | 375   | 1  | 0.5  | 0.27/62/1.4 |
| 11                  | 15   | 520 | 5100 | 365   | 1  | 0.56 | 0.16/57/2.8 |
| Comparative Example |      |     |      |       |    |      |             |
| 4                   | 14   | 860 | —    | —     | 1  | 0.3  | —/60/3.2    |
| 5                   | 56   | 220 | 1050 | 19    | 1  | 0.4  | 0.3/59/1.1  |
| 6                   | 13.3 | 221 | 1200 | 90    | 1  | 0.43 | 0.21/56/3.8 |

## EXAMPLE 12

One hundred parts of the resin of Example 1 having been crushed into sizes passing through a mask of 2 mm in opening was blended with 65 parts of magnetic particles (Magnetite EPT 1000 produced by Toda Kogyo K. K.), 2 parts of a metal complex dye (E-81 produced by Orient Kagaku K. K.) as a charge controller agent, and 4 parts of low-molecular weight polypropylene (Viscol 660P produced by Sanyo Kasei Kogyo K. K.) by means of a Henschel mixer, and kneaded on a roll mil under 50 melting.

After cooling, the mixture was coarsely crushed by means of a hammer mil and then pulverized by means of an ultrasonic jet pulverizer. The produce was then classified by a wind power classifier to collect particles 55 with sizes in the range of 5-35 $\mu$ . With 100 parts of the particles thus collected, 0.4 part of hydrophobic colloidal silica powder was mixed to give a toner, which was then used for image formation.

For the image formation, a commercially available 60 plain paper copier (NP-500RE produced by Canon K. K.) and the resultant toner image was fixed on a prescribed copy paper by means of hot rollers of standard specification.

The copied image obtained was good without fog in 65 the initial stage of a successive copying test and also was sufficiently good even after 20,000 sheets of a running test. After the test, no damage nor fusion sticking of the

toner was observed at the photosensitive drum, the cleaning unit and the developing sleeve.

The toner showed an excellent fixability which was of no problem even in 50,000 sheets of a running test, in which no jamming was caused by wrapping of paper onto rollers in the stage of paper discharge. Thus, the toner was satisfactory as a whole. Further, in a start-up and continuous copying test in the environment of 10° C., no trouble was caused by insufficient fixability. On the other hand, undesirable offsetting did not occur even when a part of hot fixation rollers reached a temperature of above 200° C.

## EXAMPLE 13

Example 12 was repeated except that 100 parts of the resin of Example 3 was used, whereby similarly good results were obtained as in Example 12.

## EXAMPLES 14-17, COMPARATIVE EXAMPLES 7-10

Example 12 was repeated except that the resin was replaced as shown in the following Table 3A. The results are shown in Table 3B together with those of Examples 12 and 13.

TABLE 3A

|                     | Resin                             | magnetic powder   | charge controller | release agent |
|---------------------|-----------------------------------|-------------------|-------------------|---------------|
| Example             |                                   |                   |                   |               |
| 12                  | Example 1 (100 parts)             | ETP-1000 65 parts | E-81 2 parts      | 660-P 4 parts |
| 13                  | Example 3 (100 parts)             | ETP-1000 65 parts | E-81 2 parts      | 660-P 4 parts |
| 14                  | Example 4 (100 parts)             | ETP-1000 65 parts | E-81 2 parts      | 660-P 4 parts |
| 15                  | Example 7 (100 parts)             | ETP-1000 65 parts | E-81 2 parts      | 660-P 4 parts |
| 16                  | Example 8 (100 parts)             | ETP-1000 65 parts | E-81 2 parts      | 660-P 4 parts |
| 17                  | Example 10 (100 parts)            | ETP-1000 65 parts | E-81 2 parts      | 660-P 4 parts |
| Comparative Example |                                   |                   |                   |               |
| 7                   | Comparative Example 1 (100 parts) | ETP-1000 65 parts | E-81 2 parts      | 660-P 4 parts |
| 8                   | Comparative                       | ETP-1000          | E-81              | 660-P         |

TABLE 3A-continued

|    | Resin                                | magnetic powder | charge controller | release agent |
|----|--------------------------------------|-----------------|-------------------|---------------|
| 9  | Example 2<br>(100 parts)             | 65 parts        | 2 parts           | 4 parts       |
|    | Comparative Example 3<br>(100 parts) | ETP-1000        | E-81              | 660-P         |
| 10 | Comparative Example 4<br>(100 parts) | ETP-1000        | E-81              | 660-P         |
|    | Comparative Example 6<br>(100 parts) | 65 parts        | 2 parts           | 4 parts       |
| 11 | Comparative Example 6<br>(100 parts) | ETP-1000        | E-81              | 660-P         |
|    |                                      | 65 parts        | 2 parts           | 4 parts       |

TABLE 3B

|                            | Developing durability | Fogging  | Toner M.I. *1 | Minimum fixable temp. *2 | Offset generation temp. |
|----------------------------|-----------------------|----------|---------------|--------------------------|-------------------------|
| <u>Example</u>             |                       |          |               |                          |                         |
| 12                         | 20,000 sheets<br>Good | None     | 1.8           | 135° C.                  | above 200° C.           |
| 13                         | 20,000 sheets<br>Good | None     | 1.2           | 140                      | above 200° C.           |
| 14                         | 20,000 sheets<br>Good | None     | 1.0           | 140                      | above 200° C.           |
| 15                         | 20,000 sheets<br>Good | None     | 2.2           | 135                      | above 200° C.           |
| 16                         | 20,000 sheets<br>Good | None     | 1.5           | 135                      | above 200° C.           |
| 17                         | 20,000 sheets<br>Good | None     | 1.2           | 140                      | above 200° C.           |
| <u>Comparative Example</u> |                       |          |               |                          |                         |
| 7                          | 20,000 sheets<br>Good | None     | 1.4           | 150                      | 195° C.                 |
| 8                          | 20,000 sheets<br>Good | None     | 1.1           | 145                      | 190° C.                 |
| 9                          | *3                    | Not good | 4.8           | 130                      | 180                     |
| 10                         | 20,000 sheets<br>Good | None     | 2.8           | 140                      | 180                     |
| 11                         | 20,000 sheets<br>Good | None     | 3.4           | 135                      | 180                     |

\*1: The toner M.I. was measured under the conditions of 125° C., 10 kg.

\*2: The fixability was evaluated by using the fixer of a copier NP-400RE (produced by Canon K.K.) with modification so as to be set at variable temperatures.

\*3: Image density decreased during durability test.

What is claimed is:

1. A binder resin for a toner comprising a polymer having at least three peaks or shoulders in its chromatogram obtained by gel permeation chromatography, wherein said at least three peaks or shoulders include a peak or shoulder A having the smallest molecular weight  $M_a$  of 2,000 to 80,000, a peak or shoulder C having the largest molecular weight  $M_c$  of  $3 \times 10^6$  or larger satisfying the relationship of  $M_c/M_a \geq 150$ , and a peak or shoulder B having an intermediate molecular weight  $M_b$  between said  $M_a$  and  $M_c$  of  $3 \times 10^5$  to  $1 \times 10^6$ , wherein said peaks or shoulders A, B and C have heights  $H_a$ ,  $H_b$  and  $H_c$ , respectively, which satisfy the proportion  $H_a:H_b:H_c$  of 1:0.2-1.0:0.1-0.6.

2. The binder resin according to claim 1, wherein said peak or shoulder B has a molecular weight  $M_b$  of  $3 \times 10^5$  to  $1 \times 10^6$ .

3. The binder resin according to claim 1, wherein said peak or shoulder C has a molecular weight of  $3 \times 10^6$  or larger.

4. The binder resin according to claim 1, wherein said peaks or shoulders A, B and C have heights  $H_a$ ,  $H_b$  and  $H_c$ , respectively, satisfying the proportional relationship of  $H_a:H_b:H_c$  of 1:0.2-1.0:0.1-0.6.

5. The binder resin according to claim 1, wherein the molecular weight  $M_a$  is 2,000 to 40,000.
6. The binder resin according to claim 1, wherein said polymer is a vinyl polymer.
- 5 7. The binder resin according to claim 1, which comprises a mixture of a plurality of polymers, said plurality of polymers in combination giving said at least three peaks in the chromatogram.
8. The binder resin according to claim 1, wherein said polymer has a melt index of 0.25 to 5.
9. The binder resin according to claim 1, wherein said polymer has a softening point of from 100° to 150° C.
10. The binder resin according to claim 1, wherein said polymer has a glass transition point of from 40 to 80° C.
11. The binder resin according to claim 1, wherein the polymer is contained in the binder in an amount of 60% or more by weight.
12. A toner composition for development, comprising 20 a colorant and a binder resin, said binder resin comprising a polymer having at least three peaks or shoulders in its chromatogram obtained by gel permeation chromatography, wherein said at least three peaks or shoulders include a peak or shoulder A having the smallest molecular weight  $M_a$  of 2,000 to 80,000, a peak or shoulder C having the largest molecular weight  $M_c$  of  $3 \times 10^6$  or larger satisfying the relationship of  $M_c/M_a \geq 150$ , and a peak or shoulder B having an intermediate molecular weight  $M_b$  between said  $M_a$  and  $M_c$  of  $3 \times 10^5$  to  $1 \times 10^6$  wherein said peaks or shoulders A, B and C have heights  $H_a$ ,  $H_b$ , and  $H_c$ , respectively, which satisfy the proportion  $H_a:H_b:H_c$  of 1:0.2-1.0:0.1-0.6.
13. The toner composition according to claim 12, wherein said peak or shoulder B has a molecular weight 35  $M_b$  of  $3 \times 10^5$  to  $1 \times 10^6$ .
14. The toner composition according to claim 12, wherein said peak or shoulder C has a molecular weight of  $3 \times 10^6$  or larger.
15. The toner composition according to claim 12, 40 wherein said peaks or shoulders A, B and C have heights  $H_a$ ,  $H_b$  and  $H_c$ , respectively, satisfying the proportional relationships of  $H_a:H_b:H_c$  of 1:0.2 to 1.0:0.1 to 0.6.
16. The toner composition according to claim 12, 45 wherein the molecular weight  $M_a$  is 2,000 to 40,000.
17. The toner composition according to claim 12, wherein said polymer is a vinyl polymer.
18. The toner composition according to claim 1, 50 which comprises a mixture of a plurality of polymers, said plurality of polymers in combination giving said at least three peaks in the chromatogram.
19. The toner composition according to claim 12, wherein said polymer has a melt index of 0.25 to 5.
20. The toner composition according to claim 12, 55 wherein said polymer has a softening point of from 100° to 150° C.
21. The toner composition according to claim 12, wherein said polymer has a glass transition point of from 40° to 80° C.
22. A process for producing a binder resin according to claim 1, comprising: subjecting a mixture of a vinyl monomer and a crosslinking monomer to suspension polymerization in an organic solvent capable of dissolving the polymerization product of the mixture in the presence of a polymerization initiator having a 10 hour-half life temperature of 100° C. or higher.
23. The process according to claim 22, wherein said vinyl monomer is selected from the group consisting of

styrene,  $\alpha$ -methylstyrene, p-chlorostyrene, acrylic acid, methyl acrylate, ethyl acrylate, butyl acrylate, dodecyl acrylate, octyl acrylate, phenyl acrylate, methacrylic acid, methyl methacrylate, ethyl methacrylate, butyl methacrylate, octyl methacrylate, acrylonitrile, acrylamide, maleic acid, monobutyl maleate, dibutyl maleate, monomethyl maleate, dimethyl maleate, vinyl chloride, vinyl acetate, vinyl benzoate, vinyl methyl ketone, vinyl ethyl ketone, vinyl methyl ether, vinyl ethyl ether, vinyl isobutyl ether, and a mixture thereof.

24. The process according to claim 22, wherein said crosslinking monomer is a compound having two or more polymerizable double bonds.

25. The process according to claim 23, wherein said crosslinking monomer is a compound selected from the group consisting of divinylbenzene, divinylnaphthalene, ethylene glycol diacrylate, ethylene glycol dimethacrylate, 1,3-butanediol dimethacrylate, divinylaniline, divinyl ether, divinyl sulfide, divinyl sulfone, and a mixture thereof.

26. The process according to claim 22, wherein said polymerization initiator is selected from the group consisting of 1,1-(t-butylperoxy)-3,3,5-trimethylcyclohexane, n-butyl-4,4-di-(t-butylperoxy)valerate, dicumyl peroxide,  $\alpha, \alpha'$ -bis(t-butylperoxydiisopropyl)benzene, 25 t-butylperoxycumene, di-t-butylperoxide, and diazoaminoazobenzene.

27. The process according to claim 22, wherein said solution polymerization is carried out at a temperature higher than the 10 hour-half life temperature of the 30 polymerization initiator by 0°-40° C.

28. The toner according to claim 12, wherein the polymer is contained in the binder resin in an amount of 60% or more by weight.

29. A process for producing a binder resin for toner, comprising uniformly mixing a polymer having a weight-average molecular weight of  $1 \times 10^3$  to  $8 \times 10^4$ , a polymer having a weight-average molecular weight of  $3 \times 10^5$  to  $10^6$  and a polymer having a weight-average molecular weight of  $3 \times 10^6$  or larger, to form a polymer mixture having at least three peaks or shoulders in its chromatogram obtained by gel permeation chromatography, wherein said at least three peaks or shoulders include a peak or shoulder A having the smallest molec-

ular weight Ma of 2,000 to 80,000, a peak or shoulder C having the largest molecular weight Mc satisfying, the relationship of  $Mc/Ma \geq 150$ , and a peak or shoulder B having an intermediate molecular weight between said 5 Ma and Mc.

30. The process according to claim 29, wherein the mixing of the polymers are carried out by mixing the polymers each in solution, and the solvent is evaporated off from the resultant solution mixture to recover the 10 polymer mixture.

31. The process according to claim 29, wherein the peak or shoulder A has a molecular weight Ma of 2,000 to 80,000, the peak or shoulder B has a molecular weight Mb of  $3 \times 10^5$  to  $1 \times 10^6$  and the peak or shoulder C has a molecular weight Mc of  $3 \times 10^6$  or larger, wherein said peaks or shoulders A, B and C have heights Ha, Hb and Hc, respectively, which satisfy the proportion Ha:Hb:Hc of 1:0.2-1.0: 0.1-0.6.

32. A process for producing a toner, comprising: melt-kneading a colorant and a binder resin, said binder resin comprising a polymer having at least three peaks or shoulders in its chromatogram obtained by gel permeation chromatography, wherein said at least three peaks or shoulders include a peak or shoulder A having the smallest molecular weight Ma of 2,000 to 80,000, a peak or shoulder C having the largest molecular weight Mc satisfying the relationship of  $Mc/Ma \geq 150$ , and a peak or shoulder B having an intermediate molecular weight between said Ma and Mc, cooling the resultant mixture, and pulverizing and classifying the cooled mixture to obtain said toner.

33. The process according to claim 32, wherein the peak or shoulder A has a molecular weight Ma of 2,000 to 80,000, the peak or shoulder B has a molecular weight Mb of  $3 \times 10^5$  to  $1 \times 10^6$  and the peak or shoulder C has a molecular weight Mc of  $3 \times 10^6$  or larger, wherein said peaks or shoulders A, B and C have heights Ha, Hb and Hc, respectively, which satisfy the proportion Ha:Hb:Hc of 1:0.2-1.0: 0.1-0.6.

34. The process according to claim 32, wherein the polymer is contained in the binder resin in an amount of 60% or more by weight.

\* \* \* \* \*

UNITED STATES PATENT AND TRADEMARK OFFICE  
CERTIFICATE OF CORRECTION

PATENT NO. : 4,626,488

Page 1 of 2

DATED : December 2, 1986

INVENTOR(S) : SUKEJIRO INOUE

It is certified that error appears in the above-identified patent and that said Letters Patent is hereby corrected as shown below:

COLUMN 2

Line 32, "decreased, or maintenance" should read  
--decreased maintenance, or maintenance--.

COLUMN 6

Line 68,  $10^6 \geq Mc \geq -5$  should read  $10^6 \leq Mc \leq -5$ .

COLUMN 7

Line 14, "15-0.4." should read --0.15-0.4--.  
Lines 52-53, "5/1 to 1/l." should read --5:1 to 1:l--.  
Line 54, "1/5." should read --1:5--.

COLUMN 10

Line 28, "carboxilic" should read --carboxylic--.

COLUMN 13

Line 51, "Toulene" should read --Toluene--.

COLUMN 15

Line 18, " Styrene-BA copolymer 70/30" should read  
--5 Styrene-BA copolymer 70/30--.

COLUMN 17

Lines 36-39, "180" should read --180°C.--.  
180  
180  
180

UNITED STATES PATENT AND TRADEMARK OFFICE  
CERTIFICATE OF CORRECTION

PATENT NO. : 4,626,488

Page 2 of 2

DATED : December 2, 1986

INVENTOR(S) : SUKEJIRO INOUE

It is certified that error appears in the above-identified patent and that said Letters Patent is hereby corrected as shown below:

COLUMN 17

Line 67, "aatisfying" should read --satisfying--.

COLUMN 18

Line 14, "40 to" should read --40° to--.

Line 62, "suspension" should read --solution--.

COLUMN 19

Line 26, "di-ti-butylperoxide" should read  
--di-t-butylperoxide--.

COLUMN 20

Line 2, "satisfying," should read --satisfying--.

Signed and Sealed this

Fifteenth Day of September, 1987

*Attest:*

DONALD J. QUIGG

*Attesting Officer*

*Commissioner of Patents and Trademarks*

UNITED STATES PATENT AND TRADEMARK OFFICE  
CERTIFICATE OF CORRECTION

PATENT NO. : 4,626,488  
DATED : December 2, 1986  
INVENTOR(S) : SUKEJIRO INOUE

It is certified that error appears in the above-identified patent and that said Letters Patent is hereby corrected as shown below:

COLUMN 8

Line 28, "over" should read --oven--.

Signed and Sealed this  
Thirty-first Day of January, 1989

*Attest:*

DONALD J. QUIGG

*Attesting Officer*

*Commissioner of Patents and Trademarks*